

## UNITED STATES PATENT OFFICE

REED P. ROSE AND ALLEN F. OWEN, OF JACKSON HEIGHTS, NEW YORK, ASSIGNORS TO  
THE MECHANICAL RUBBER COMPANY, OF CLEVELAND, OHIO, A CORPORATION OF  
NEW JERSEY

## METHOD OF MAKING FIBER-RUBBER MATERIAL

No Drawing.

Application filed August 11, 1927. Serial No. 212,356.

This invention relates to a fiber-rubber material and the method of making the same, more particularly to a leather substitute suitable for uses similar to those in which sole leather is employed.

Leather of the "sole leather" type has a wide use in the arts, more particularly for shoe parts such as soles and doublers, counters and toe boxes, belting, gaskets, pump valves and cups, shims such as body shims for automobiles and many other purposes. However, leather of this character is relatively expensive, since for the highest class articles only selected parts of the best grade hides can be used. Moreover, while sole leather has many desirable qualities which fit it for the above and other purposes, it is open to a number of objections the most important of which is lack of uniformity which is apparent not only between different lots but to a great extent even in the individual hides. While its tensile strength and resistance to flexing and abrasion are relatively good, there is room for considerable improvement in these respects, and it is also open to the objection that it is water absorbent, and when water soaked, it loses its resistance to abrasion and cutting and loses in tensile strength, and it has the further disadvantage that after drying, it becomes unduly stiff and does not recover its original physical characteristics. Furthermore, it deteriorates in the presence of strong alkalies and acids, and hence cannot be used for purposes where resistance to these is required.

An object of our invention is to provide a uniformly dense, tough, high tensile, flexible, water and abrasion resistant composition of fiber and rubber. Another object is to provide a sole leather substitute which can be used for every purpose for which sole leather is now used having properties substantially equaling or surpassing those of genuine leather. Another object is to provide a finished shoe bottoming blank directly from an aqueous suspension of fiber and rubber. A further object is to provide shoe soles, doublers, counters, toe boxes and other findings of improved quality and to provide an inexpensive method of manufacturing the

same. A still further object is to provide a method of preparing and treating the composition by which the desired qualities are obtained. Further objects will appear from the detailed description and claims.

55

The invention consists broadly in a fiber-rubber material comprising a closely matted mass of fibers firmly bonded by small substantially discontinuous particles deposited from an aqueous dispersion of rubber either alone or compounded, the material being characterized by its density, toughness, high tensile and high flexing test, and resistance to water and abrasion. The invention further comprises the method for making the

65

material.

In carrying out the invention, an aqueous suspension of fiber mixed with an aqueous dispersion of rubber is first prepared. While it is preferred to use vegetable fibers such as cotton any other fiber or mixtures thereof possessing the desired characteristics may be used. The cotton or other fiber is first partly hydrolyzed in any suitable manner preferably by treating with water in any suitable type of a heating engine or hollander. The beating operation is carried out with care so that the fibers are drawn or brushed out and not cut fine and is continued until the fiber has been hydrolyzed to such an extent

75

that the fiber surfaces have been reduced to a gelatinous condition. Any suitable aqueous dispersion of rubber, such as natural latex, unvulcanized or vulcanized, or an artificial dispersion of rubber, is then added to the above prepared aqueous suspension of fiber. The invention also includes the addition, if desired, of any suitable compounding or filling ingredients including protective colloids such as glue, treated starches, casein, etc. and any other ingredients by which it is desired to modify the properties.

80

After the batch is thoroughly mixed, the rubber from the aqueous dispersion is then deposited in particles of substantially microscopic size upon the individual fibers either by a slow continuous coagulation, or by adding the coagulant in two stages so as to first produce an agglomeration of the rubber particles on the fiber, followed by a subsequent

95

100

coagulation. It is preferred to utilize the two-stage method of depositing the rubber on the fiber. It is preferable when making a shoe bottoming material to use an amount of the rubber dispersion sufficient to provide 5 12-50% of rubber in the finished product, the lower percentage being the most suitable for economically making a doubler material, while higher proportions of rubber 10 are preferable for shoe soling materials.

When using the above prepared batch as a base, the material of our invention is then formed into the shape required for the finished article in any of the following ways:

- 15 The solid material of the batch may be deposited in sheet form of the desired thickness directly from the suspension in water by the use of a paper machine of the Fourdrinier or cylinder type. After the formation of a 20 sheet of suitable thickness, the wet sheet is then cold pressed preferably between the plates or platens of a press at a pressure not to exceed that at which the sheet will flow or spread while in its wet condition. The main 25 purpose of this pressing is to remove moisture and to initially consolidate or compact the material. The pressure used can be between the limits of 50 to 500 lbs., but for the higher pressures it is preferable to apply it gradually 30 in order not to distort the position of the fibers in the sheet and spread the same. If products of a medium quality are desired such as shoe doublers or mid-soles, counters, toe boxes and automobile body shims the 35 moisture content may be reduced to form 10-15% in one drying operation. However, if a better quality product is desired the drying 40 step should be carried to a point where the material contains between 20 and 30% moisture and should be followed by an intermediate pressing step using a pressure of from 500 to 1200 lbs. per square inch with a cold press. After this intermediate pressing 45 step the drying is continued until a moisture content of from 10-15% is reached. After the cold pressing the sheet is dried in any suitable manner until its moisture content has been further reduced. Following the drying step, the sheet is then 50 hot pressed at a temperature and under a pressure which will vary somewhat with conditions and the purpose for which the finished material is to be used. That is, if a relatively high heat and long 55 pressing are employed, the pressure may be somewhat reduced, while if the heat is lower and the pressing of comparatively short duration, the pressure should be greater. Other things being equal, the higher the pressure 60 the greater the density, toughness, tensile strength, water and abrasion resistance of the sheet, but if the pressure is unduly high, the flexibility may be decreased to such an extent that the material is no longer suitable 65 for shoe bottoming purposes requiring

considerable flexibility but may be used for other purposes where flexibility is not an essential factor. The pressure should not be substantially below 800 lbs. in the making of a sole or doubler material, and by reason of the aforesaid decrease in flexibility, it should not substantially exceed 2000 lbs., the preferred limits for the pressing being from about 1200 to 2000 lbs. at a temperature of from 225° F. to 310° F. for these products. 70 While, if desired, vulcanizing ingredients may be included and the material vulcanized, satisfactory results are obtained without vulcanization. After the final pressing step the material, if to be used for shoe bottoming, is then cut into the desired blanks, and in this connection it may be pointed out that the characteristics of the material are such that it may be channeled, skived, stitched or otherwise treated in the same manner as genuine leather and by the use of the same machinery. 75 Where flexibility is not a paramount requisite the pressure limits may extend beyond 2000 lbs. as for example in using the material for purposes such as pump valves, cups, etc. 80

Instead of forming the wet sheet on a continuous type of paper machine such as the Fourdrinier or cylinder type it may be built up by the use of a wet or board machine, plying up on a suitable pick up or making roll to the desired thickness, and then removing the sheet. If desired, an aqueous dispersion of rubber, such as natural or artificial rubber latex, may be sprayed or otherwise applied between the layers as they are plied up on the making roll and the latex may be compounded with glue or other suitable ingredients for the purpose of increasing or decreasing the adhesiveness, tensile strength, etc. of the dispersed rubber. If glue is used it may be set or not as desired by the use of formaldehyde, tannic acid or other suitable agent. The use of glue in this way improves the bond between the plies and also adds to the water resistance. The wet sheet as obtained from the cylinder machine may then be subjected to the same pressing and drying operations as above described in connection with the product from the continuous sheet forming machine. 105

As an alternative to either of the above methods of forming the wet sheet, it may be produced by centrifugal deposition from the suspension in the following manner:

An ordinary centrifugal may be partitioned off into compartments either vertically or horizontally by pairs of walls of finely perforated metal or other suitable material spaced sufficiently to give the desired thickness of material and opening into a common cylindrical compartment running vertically and parallel with the periphery of the basket. On supplying the machine with the fiber-rubber suspension, the material will be deposited in a sheet between the 115 120 125 130

walls. The sheet thus obtained may be pressed and dried as before described.

As a further alternative, the wet sheet may be formed by a slow filtration or vacuum filtration of the suspension on a screen or other porous media after which the wet sheet thus produced may be pressed and dried in the same manner as before described.

10 As a still further modification, a suspension of fiber and rubber, obtained as before described may be partially dehydrated by allowing it to settle or by any other suitable means and then the wet fibrous mass placed 15 in a suitable mixing apparatus, such as a Werner-Pfleiderer mixer, and an additional amount of natural or artificial latex, such as a dispersion of rubber in water with or without the addition of glue or other suitable 20 protective colloid, is added to the batch in the mixer, and the mixing operation continued until the added rubber and other ingredients are uniformly distributed throughout the mass. No coagulating step is used 25 upon the portion of the rubber added to the batch in the mixing machine and if the proper protective colloid is used, coagulation does not take place until the material is partially dried. This mixing is continued 30 until the batch is in a proper condition to be extruded through a suitable apparatus, which may be an ordinary tuber or pug mill fitted with an orifice capable of giving a 35 shape to the material approximating that desired in the finished product. The material may be cold pressed, dried with or without the intermediate pressing and then hot pressed as previously described. Alternatively, the product from the mixing machine 40 may be partially dried down to a moisture content of between 20-30% and then made into sheet or ribbon form by any suitable means.

Another method of forming a sheet is to 45 place the rubber fiber mixture between two moving convergent wires or felt surfaces built in the form of a vertical hopper so that as the body of the rubberized fiber moves toward the bottom of the machine it 50 is gradually compacted with the removal of water until the sheet coming from the bottom orifice of the machine is of desired thickness, and with a sufficiently low moisture content so that it can be handled as is 55 the case with a sheet from an ordinary Fourdrinier paper machine. This sheet is then pressed, dried and treated in every way as described above.

By our invention a leather substitute may 60 be produced which is similar in appearance to leather of the sole leather or doubler types and in which the fibrous material is distributed continuously throughout the body of the material, and is bonded by rubber either from natural latex or from an aque-

ous dispersion of rubber (crude or reclaimed) uniformly distributed in minute particle form substantially invisible to the naked eye throughout the body of the material to form a continuous fibroid flexible sheet, having the characteristic appearance of leather, especially after abrasion, being dense and tough, and having a high flexing and tensile test and a high resistance to water absorption and abrasion. Moreover, even after long exposure to moisture, it still retains its characteristic properties and is not softened, warped, mushroomed, and otherwise deteriorated as is the case with leather. It may be manipulated in the same general manner and by the same machinery as is used for leather. While it may contain a relatively high percentage of rubber, it has the general appearance and characteristics of leather and has not the rubber-like feel and appearance of a similar compound made by mixing fiber on a mill with plasticized rubber. Its resistance to abrasion is also vastly superior to that of an ordinary milled rubber-fiber compound and the abrasion is very uniform.

While a specific disclosure has been made of the invention, it is obvious that changes may be made therein without departing from its spirit, and it is therefore not desired to limit the invention more than is required by the prior art and as set forth in the appended claims.

Having thus described our invention, what we claim and desire to protect by Letters Patent is:

1. The method of forming a fiber-rubber material which comprises forming an aqueous suspension of rubber and vegetable fiber, depositing the rubber on the fiber, forming a relatively thick wet sheet material therefrom, cold pressing the material without flowing or spreading it to compact it and remove moisture, drying the material to not substantially over 15% moisture, and hot 105 pressing at an increased pressure.

2. The method of forming a fiber-rubber material which comprises forming an aqueous suspension of rubber and vegetable fiber, coagulating the rubber on the fiber, forming a relatively thick wet sheet material therefrom, cold pressing the material without flowing or spreading it to compact it and remove moisture, drying the material to not substantially over 15% moisture, and hot 115 pressing at over 800 lbs. pressure.

3. The method of forming a fiber-rubber material which comprises forming an aqueous suspension of rubber and partly hydrolyzed vegetable fiber, coagulating the rubber on the fiber, forming a relatively thick wet sheet material therefrom, cold pressing the material at not substantially over 1000 lbs. pressure, drying to not substantially over 125

- 15% moisture, and hot pressing at over 800 lbs. pressure.
4. The method of forming a fiber-rubber material which comprises forming an aqueous suspension of rubber and partly hydrolyzed vegetable fiber, coagulating the rubber on the fiber, forming a relatively thick wet sheet material therefrom, cold pressing the material at not substantially over 1000 lbs. pressure, drying to not substantially over 15% moisture, and hot pressing at 1400-2000 lbs. pressure.
5. The method of forming a fiber-rubber material which comprises forming an aqueous suspension of rubber and partly hydrolyzed vegetable fiber, coagulating the rubber on the fiber, forming a relatively thick wet sheet material therefrom, cold pressing the material without flowing or spreading it to compact it and remove moisture, drying the material to substantially 10-15% moisture, and hot pressing at 1400-2000 lbs. pressure.
6. The method of forming a fiber-rubber material which comprises forming an aqueous suspension of rubber and partly hydrolyzed vegetable fiber, coagulating the rubber on the fiber, forming a relatively thick wet sheet material therefrom, cold pressing the material at not substantially over 1000 lbs. pressure, drying to substantially 10-15% moisture, and hot pressing at not substantially over 2000 lbs. pressure.
7. The method of forming a fiber-rubber material which comprises mixing an aqueous suspension of partly hydrolyzed vegetable fiber and a sufficient amount of an aqueous suspension of rubber to provide 12-50% rubber, coagulating the rubber on the fiber, forming a relatively thick wet sheet material therefrom, cold pressing the material without flowing or spreading it to compact it and remove moisture, drying the material to not substantially over 15% moisture, and hot pressing at an increased pressure.
8. The method of forming a fiber-rubber material which comprises mixing an aqueous suspension of partly hydrolyzed vegetable fiber and a sufficient amount of an aqueous suspension of rubber to provide 12-50% rubber, coagulating the rubber on the fiber, forming a relatively thick wet sheet material therefrom, cold pressing the material at below 1000 lbs. pressure, drying the material to not substantially over 15% moisture, and hot pressing at over 800 lbs. pressure.
9. The method of forming a fiber-rubber material which comprises mixing an aqueous suspension of partly hydrolyzed vegetable fiber and a sufficient amount of an aqueous suspension of rubber to provide 12-50% rubber, coagulating the rubber on the fiber, forming a relatively thick wet sheet material therefrom, cold pressing the material without flowing or spreading it to compact it and remove moisture, drying to substan-
- tially 10-15% moisture, and hot pressing at over 1400 lbs. pressure.
10. The method of forming a fiber-rubber material which comprises mixing an aqueous suspension of partly hydrolyzed vegetable fiber with a sufficient quantity of an aqueous suspension of rubber to provide 12-50% rubber, coagulating the rubber on the fiber, forming a relatively thick wet sheet material therefrom, cold pressing the material at below 1000 lbs. pressure, drying to substantially 10-15% moisture, and hot pressing at not substantially over 2000 lbs. pressure.
11. The method of forming a fiber-rubber material which comprises mixing an aqueous suspension of vegetable fiber hydrolyzed to a partly gelatinous condition with a sufficient amount of an aqueous suspension of rubber to provide 12-50% rubber, coagulating the rubber on the fiber, forming a relatively thick wet sheet material therefrom, cold pressing the material without flowing or spreading it to compact it and remove moisture, drying to not substantially over 15% moisture, and hot pressing at over 800 lbs. pressure.
12. The method of forming a fiber-rubber material which comprises mixing an aqueous suspension of vegetable fiber hydrolyzed to a partly gelatinous condition with a sufficient amount of an aqueous suspension of rubber to provide 12-50% rubber, coagulating the rubber on the fiber, forming a relatively thick wet sheet material therefrom, cold pressing the material at below 1000 lbs. pressure, drying to substantially 10-15% moisture, and hot pressing at over 1400 lbs. pressure.
13. The method of forming shoe bottoming material which comprises forming an aqueous suspension of rubber and fiber hydrolyzed to a partly gelatinous condition, coagulating the rubber on the fiber, forming a relatively thick wet sheet therefrom, drying the sheet to not substantially over 30% moisture, cutting out shoe bottoming articles from the sheet, cold mold pressing the articles at not substantially over 1000 lbs. pressure, drying to not substantially over 15% moisture, and hot pressing at not substantially over 2000 lbs.
14. The method of forming shoe bottoming material which comprises mixing an aqueous suspension of vegetable fiber hydrolyzed to a partly gelatinous condition with a sufficient quantity of an aqueous suspension of rubber to provide 12-50% rubber, coagulating the rubber on the fiber, forming a relatively thick wet sheet therefrom, drying the sheet to not substantially over 30% moisture, cutting out shoe bottoming articles from the sheet, cold mold pressing at not substantially over 1000 lbs. pressure, drying to substantially 10-15% moisture, and hot pressing at a pressure of 1400-2000 lbs.
15. The method of manufacturing a fiber-rubber material which comprises forming a

wet sheet of intimately intermingled rubber particles and fibers, pressing the wet sheet at room temperature without spreading it, drying the wet sheet to a moisture content of not over 15%, and pressing and completely drying the sheet at an elevated temperature.

16. The method of forming a fiber-rubber material which comprises mixing an aqueous suspension of partly hydrolyzed vegetable fiber and rubber latex, coagulating the rubber on the fiber, mixing therewith a rubber latex in the presence of a protective colloid, forming an article therefrom, partially dehydrating the material, cold pressing under moderate pressure, further dehydrating, and hot pressing under a higher pressure.

17. The method of manufacturing a fiber-rubber material which comprises forming a watery body of partly hydrolyzed vegetable fibers intimately associated with coagulated rubber particles, mixing therewith a water suspension of rubber in the presence of a protective colloid, shaping an article therefrom, partially dehydrating, cold pressing, further dehydrating, and hot pressing under a higher pressure.

18. As a new article, a fiber-rubber material comprising a dense, compressed, relatively thick, flexible sheet of closely matted relatively long vegetable fibers, the individual fibers being spaced and strongly united by a relatively thin bond of gelatinized hydrated cellulose and the deposition product of an aqueous rubber dispersion.

35 Signed at New York, county and State of New York, this 5th day of August, 1927.

REED P. ROSE.

Signed at Cleveland, county of Cuyahoga and State of Ohio, this 8th day of August, 40 1927.

ALLEN F. OWEN.

45

50

55

60

65